

# UNITED STATES PATENT OFFICE.

TATSUZO KOSUGI, OF SEIDO-MURA, KOBE, JAPAN.

## ALLOY.

1,369,818.

Specification of Letters Patent.

Patented Mar. 1, 1921.

No Drawing.

Application filed June 30, 1920. Serial No. 393,209.

*To all whom it may concern:*

Be it known that I, TATSUZO KOSUGI, a subject of the Emperor of Japan, residing in Seido-mura, county of Muko, Prefecture 5 of Kobe, Japan, have invented certain new and useful Improvements in Alloys, of which the following is a specification.

The present invention relates to an alloy comprising copper, aluminium, nickel and iron and has for its object to obtain an alloy having a great tensile strength, not easily susceptible of corrosive action of air or brine. Another object is to obtain an alloy in which blow holes and flaws are not produced by casting and forging operations.

In the present invention I use copper in preponderating amount, together with aluminium, nickel and iron.

I first mix nickel and iron in a crucible, 20 melting them by heating, and then I add copper to the molten mass. After heating the mixture for a while I add aluminium thereto. When the whole matter is melted, the molten mass is poured into molds to form 25 objects of any desired shape, as in ordinary metal casting.

Preferably alloys of the quaternary type may contain from one to six per cent. iron, two to seven per cent. nickel, seven to twelve 30 per cent. aluminium, with the balance copper.

The alloys prepared in this ratio give a tensile strength as high as 48 tons per square inch, a ductility of 25%, always have a homogeneity of structure, no blow holes or 35 flaws will be produced by any kind of treatment, such as casting, swaging, rolling, etc., and they will never rust but permanently retain a golden luster.

This alloy, having the excellent characteristics mentioned above, is of exceptional utility in its employment for all kinds of industrial and domestic purposes, being particularly adapted to propellers, hydraulic machines; cutting tools, furniture and decorative articles, and several operating and 45 wearing parts of engines and motors.

Having now particularly described and ascertained the nature of my said invention and in what manner the same is to be performed, I declare that what I claim is:—

An alloy, comprising seventy-five to ninety per cent. copper, seven to twelve per cent. aluminium, two to seven per cent. nickel, and one to six per cent. iron.

In witness whereof, I have hereunto signed my name in the presence of two subscribing witnesses.

TATSUZO KOSUGI.

Witnesses:

HIDEO KAI,  
M. W. SMITH.